

## UNITED STATES PATENT OFFICE.

RAY P. PERRY, OF UPPER MONTCLAIR, NEW JERSEY, ASSIGNOR TO THE BARRETT COMPANY, A CORPORATION OF NEW JERSEY.

## PRODUCTION OF BUILDING FELT.

No Drawing.

Application filed April 7, 1922. Serial No. 550,469.

This invention relates to the production of felts and the like. It relates more particularly to the production of products that are especially suitable for such uses as roofing strips and shingles.

5 An object of the invention is to produce products of this character having incorporated therein, during the course of its manufacture, a proportion of waterproofing material which can be varied in amount throughout a wide range without interfering with the continuity of operation of the process and without departing from the spirit or scope of this invention.

10 Another object of the invention is to render it possible to produce such products having incorporated therein a materially larger percentage of waterproofing material than has heretofore been feasible with the old processes as used in practice.

15 Another object is to overcome the difficulties that have heretofore been experienced when it was attempted to introduce a large percentage of waterproofing material into such products when the cheap or relatively inexpensive fibrous materials were used in making the same. Other objects and advantages of the invention will be obvious as the description proceeds.

20 In practicing this invention an aqueous emulsion of the waterproofing material, which it is desired to use, may be mixed with fibrous material in the beaters of an ordinary paper-making machine and becomes incorporated in the sheet while the sheet is being formed. The waterproofing material to be used may, for example, be pitch or asphalt, and its melting point may vary to a considerable extent, say from about 100° F. or lower to 200° F. or higher. The fibrous material to be used may be ordinary waste paper stock or a mixture of waste paper stock and rag stock, etc.

25 An aqueous emulsion of the waterproofing material, such as pitch or asphalt, may be made for example by introducing the waterproofing material into water containing an emulsifying agent, such an agent being a water-containing silicate that occurs in nature and has a hardness of less than 3 and usually a hardness of from 1 to 2. Steatite, e. g. talc or soapstone is an example of the type of the emulsifying agent which I may use. The emulsifying agent will be finely ground or pulverized and the proportions

30 may vary throughout a wide range. The mixture of water, emulsifying agent, and waterproofing material may be stirred or violently agitated, if necessary, to insure thorough emulsification. A satisfactory sheet may be obtained by mixing the emulsion with a sufficient amount of paper or felt-making material, so that the final water-free sheet will consist of about 50% more or less by weight of fibrous material together with 65 waterproofing material and the emulsifying agent in the proportions ranging from about 10 to 1 of the latter materials to the proportion of about 1 to 4 of the same, the combined weight of the waterproofing and emulsifying materials generally being less than half 70 of the weight of the sheet.

75 A water pulp of fibrous material may be mixed with the aqueous emulsion of bituminous or waterproofing material and soapstone or other emulsifying agent before the emulsion is introduced into the vat of a paper-making machine. Or the paper-making fibrous material may be introduced into an emulsion of waterproofing material, and the 80 mixture then introduced into the vat of the paper-making machine. By following this procedure small particles of waterproofing material are intermingled with the fibers of the paper pulp, so that as the sheet is formed 85 on the paper-making machine, the particles of waterproofing material become substantially uniformly distributed throughout the sheet with the fibers.

90 After the sheet containing the fibers and the particles of waterproofing material has been formed, it may be dried by means of drying rolls, or it may be air dried. Instead of drying the sheet as mentioned, the sheet may be passed between pressure rolls, which 95 rolls may, if desired, be hot, so that a part drying and a part pressing operation will take place.

100 It is obvious that the sheets formed as described may be passed through a saturating bath and may then be coated in the usual way for roofing purposes. The sheets may also be plied together either before or after drying the same, and heat and pressure may be thereafter used in order to join the sheets, 105 together and make a substantially homogeneous and uniform thick sheet.

I claim:

110 1. The herein described process, which comprises mixing in water, paper-making

- stock and an emulsion containing waterproofing material and steatite, and forming on a paper-making machine a sheet from said mixture.
5. The herein described process, which comprises mixing in water, paper-making stock and an emulsion containing bituminous waterproofing material and steatite, and forming on a paper-making machine a sheet from said mixture.
10. The herein described process, which comprises mixing in water, paper-making stock and an emulsion containing asphalt and steatite, and forming on a paper-making machine a sheet from said mixture.
15. The herein described process, which comprises mixing in water, paper-making stock and an emulsion containing asphalt and steatite in substantially the proportions of 5 to 1, and forming on a paper-making machine a sheet from said mixture.
20. The herein described process, which comprises mixing in water, paper-making stock and an emulsion containing waterproofing material and soapstone, and forming on a paper-making machine a sheet from said mixture.
25. The herein described process, which comprises mixing in water, paper-making stock and an emulsion containing asphalt and soapstone, and forming on a paper-making machine a sheet from said mixture.
30. The herein described process, which comprises mixing in water, paper-making stock and an emulsion containing bituminous waterproofing material and soapstone, and forming on a paper-making machine a sheet from said mixture.
35. The herein described process, which comprises mixing in water, paper-making stock and an emulsion containing asphalt and soapstone, and forming on a paper-making machine a sheet from said mixture.
40. The herein described process, which comprises mixing in water, paper-making stock and an emulsion containing asphalt and soapstone in substantially the proportions of 5 to 1, and forming on a paper-making machine a sheet from said mixture.
45. The herein described process, which comprises mixing in water, paper-making stock and an emulsion containing asphalt and soapstone in substantially the proportions of 5 to 1, said mixture being in the proportion of about 10 to 40 parts by weight of stock to about 90 to 60 parts by weight of asphalt and soapstone, and forming on a paper-making machine a sheet from said mixture.
50. The herein described process, which comprises mixing in water, paper-making stock and an emulsion containing waterproofing material and talc, and forming on a paper-making machine a sheet from said mixture.
55. The herein described process, which comprises mixing in water, paper-making stock and an emulsion containing waterproofing material and talc, and forming on a paper-making machine a sheet from said mixture.
60. The herein described process, which comprises mixing paper-making stock in water with an emulsion containing bituminous waterproofing material and talc, and forming on a paper-making machine a sheet from said mixture.
65. The herein described process, which comprises mixing paper-making stock in water with an emulsion containing asphalt and talc, and forming on a paper-making machine a sheet from said mixture.
70. The herein described process, which comprises mixing paper-making stock in water with an emulsion containing asphalt and talc in substantially the proportions of 5 to 1, and forming on a paper-making machine a sheet from said mixture.
75. The herein described process, which comprises mixing paper-making stock in water with an emulsion containing asphalt and talc in substantially the proportions of 5 to 1, said mixture being in the proportion of about 10 to 40 parts by weight of stock to about 90 to 60 parts of asphalt and talc, and forming on a paper-making machine a sheet from said mixture.
80. The herein described process, which comprises mixing paper-making stock in water with an emulsion containing asphalt and talc in substantially the proportions of 5 to 1, said mixture being in the proportion of about 10 to 40 parts by weight of stock to about 90 to 60 parts of asphalt and talc, and forming on a paper-making machine a sheet from said mixture.
85. The process which comprises forming an emulsion of water, waterproofing material and talc, mixing paper-making stock therewith, and forming on a paper-making machine a sheet from said mixture.
90. The process which comprises forming an emulsion of water, waterproofing material and soapstone, mixing paper-making stock therewith, and forming on a paper-making machine a sheet from said mixture.
95. The process which comprises forming an emulsion of water, waterproofing material and steatite, mixing paper-making stock therewith, and forming on a paper-making machine a sheet from said mixture.
100. The process which comprises forming an emulsion of water, waterproofing material and steatite, mixing paper-making stock therewith, and forming on a paper-making machine a sheet from said mixture.
105. The herein described process, which comprises mixing in water, paper-making stock and an emulsion containing waterproofing material and steatite of a hardness of approximately 1, and forming on a paper-making machine a sheet from said mixture.
110. A construction material comprising fibrous material, an emulsified waterproofing material and an emulsifier consisting of steatite.
115. A construction material comprising fibrous material, an emulsified waterproofing material and an emulsifier consisting of talc.
120. A construction material comprising approximately 50% fibrous material, an emulsified waterproofing material and an emulsifier consisting of steatite.
125. A construction material comprising approximately 50% material, an emulsified waterproofing material and an emulsifier consisting of talc.
- In testimony whereof I affix my signature.
- RAY P. PERRY.

**CERTIFICATE OF CORRECTION.**

**Patent No. 1,707,491.**

**Granted April 2, 1929, to**

**RAY P. PERRY.**

**It is hereby certified that error appears in the printed specification of the above numbered patent requiring correction as follows: Page 1, line 105, after the word "sheets" strike out the comma; page 2, line 13, claim 3, before the word "an" insert the word "and"; same page, line 61, claim 11, strike out the article "a"; page 2, line 119, claim 22, before the word "material" insert the word "fibrous"; and that the said Letters Patent should be read with these corrections therein that the same may conform to the record of the case in the Patent Office.**

**Signed and sealed this 28th day of May, A. D. 1929.**

**(Seal)**

**M. J. Moore,  
Acting Commissioner of Patents.**